

March 29, 1932.

W. C. HAMPTON

1,851,509

METHOD OF COATING ARTICLES WITH PYROXYLIN

Filed Oct. 28, 1929



Inventor

William C. Hampton  
By J. D. Walker  
Attorney

## UNITED STATES PATENT OFFICE

WILLIAM C. HAMPTON, OF DAYTON, OHIO, ASSIGNOR TO THE CRAWFORD, McGREGOR AND CANBY COMPANY, OF DAYTON, OHIO, A CORPORATION OF OHIO

## METHOD OF COATING ARTICLES WITH PYROXYLIN

Application filed October 28, 1929. Serial No. 402,832.

This invention relates to a method of coating articles of metal, wood or other material with a covering of celluloid or of pyroxylin applied in a liquid form and subsequently 5 cured thereon to afford a continuous, one-piece, adherent covering of substantially uniform thickness and possessing a smooth and highly polished surface.

While reference is made in some prior 10 patents to proposed applications of celluloid or pyroxylin as a coating material by dipping articles in a body of the material in liquid form, such suggestions have been prophetic only and the necessary teaching 15 for successful working of nitrocellulose materials in liquid form has been entirely lacking. Great difficulty is encountered in controlling the material subsequent to the dipping operation and in effecting a curing of 20 the coating which will leave the finished surface undistorted and unblemished. Many unusual problems have been presented in effecting a uniformly smooth, polished surface deposit for which the hereinafter stated 25 method affords a commercially practical solution.

The solvents employed in reducing pyroxylin and celluloid to liquid form are highly volatile, evaporating rapidly and permitting the material to "set" quickly upon withdrawal from the dipping bath. Such rapid evaporation produces a refrigerating effect, causing precipitation of moisture from the surrounding atmosphere upon the coated 30 surface. If such moisture condensation trickles in streams upon the newly coated surface, it produces streaks and discoloration as well as distortion and a rough or matte surface. If such condensation stands in the 35 form of dew, ice crystals, or drops upon the freshly coated surface, it produces a rough and pitted surface effect. If the outer surface of the deposit is permitted to "set" too quickly, it forms an impenetrable film which 40 prevents the escape of solvent from the inner strata and by un-uniform shrinkage of such outer surface film upon the inner material while yet in a soft condition, it induces 45 wrinkling and produces a crinkled surface of intricate design. If the freshly coated body 50

is maintained at a moderate temperature sufficient to effect rapid evaporation of the solvent before such surface film can form, the solvent is quite likely to "boil" or vaporize within the deposit of coating material, thus forming pimples and bubbles and causing the material to swell or "balloon" often assuming odd and grotesque shapes. From the experience of many such failures, the hereinafter 55 method or process of successful treatment of articles by dipping in liquid pyroxylin or celluloid has been evolved.

The object of the present invention is to provide a comparatively simple, economical, and commercially practical method for covering various articles of wood, metal and other materials, such as steering wheels for automobiles, door knobs, handles for cutlery, golf club heads and shafts, bathroom fixtures, toilet seats, and numerous other articles of 60 everyday commercial and household use with a covering of celluloid or pyroxylin having a uniformly smooth surface possessing a natural high polish or luster without the necessity of mechanical polishing or finishing operation, and of increased durability 65 and capable of withstanding hard usage and wear, and which will provide a continuous one-piece covering without seams or joints, completely sealing the enclosed body against 70 entrance of moisture or attack by vapors or the like.

A further object of the invention is to provide an improved method or process of applying celluloid and pyroxylin in liquid form 75 and controlling the resulting deposit to prevent "watering" from rapid evaporation, pitting or eggshell surface affect from dew or ice crystal deposits of moisture condensation, pimpling and bubble formation as result of "boiling" or vaporization of the contained solvent, and wrinkling or orange peel affect due to un-uniform shrinkage.

A further object of the invention is to provide a method and process by which various articles may be coated with celluloid or pyroxylin of various colors, giving to the articles pleasing and ornamental color affects.

A further object of the invention is to provide a method or process of encasing articles

within a covering of celluloid or pyroxylin of greater or less thickness, the extent of which may be controlled at will, and which may be deposited many times deeper than that of other finishing materials such as 5 paints, lacquers, and varnishes.

A further object of the invention is to provide a protective coating upon articles of wood, metal, and other material which will be 10 tightly adherent, forming substantially a homogeneous body but which will at the same time possess sufficient flexibility to prevent cracking, chipping, crazing, and fracture.

A further object of the invention is to provide 15 a coating or covering material which, when applied to articles possessing a degree of flexibility or resiliency such as shafts or golf clubs, canes, umbrella handles and the like, will yield in unison with the coated article.

With the above primary and other incidental objects in view, as will more fully appear in the specification, the invention consists of the steps and procedure, the apparatus and 25 the method of operation or their equivalents as hereinafter described and set forth in the claims.

The accompanying drawing more or less diagrammatically illustrates the apparatus 30 for carrying out the present process, and the successive steps and stages of the method.

In carrying out the present process, any suitable solvent for pyroxylin or for celluloid such as ether, alcohol, acetate, or the like, 35 may be used. However, acetone is the best known and preferable solvent for this purpose. The process consists of two major operations, to wit, first the preparation and application of a solution of pyroxylin, and second the evaporation of the solvent while governing such evaporation by temperature control, and by preconditioning the air in which the setting or curing of the material is effected.

Preparatory to the dipping or coating operation, the pyroxylin or celluloid, as the case may be, is thoroughly dissolved in a suitable solvent until the material becomes a viscous heavy liquid. This mixing of the material 40 and the initial coating or dipping operation are best and preferably performed in a room of normal temperature of approximately seventy degrees Fahrenheit. The viscous dipping solution takes approximately the same temperature or one somewhat lower, due to the refrigerating effect of evaporation. In the accompanying drawing the preparation and dipping room is indicated as 1 in which is located the tank or vat 2 containing the acetone solution of pyroxylin, the viscosity of which is approximately of the consistency of a cake batter or a thick molasses. This liquid pyroxylin, which as approximately seventy degrees Fahrenheit is sufficiently viscous 45 to be a slow flowing liquid, will become solidi-

fied into a plastic having considerable resistance to movement at lower temperature.

The article to be coated, whether it be an automobile steering wheel, a golf club shaft or head, a door knob, a toilet seat or other articles, is dipped rather slowly into this viscous liquid to prevent carrying air bubbles into the liquid, and is then slowly withdrawn. The dipped article is held momentarily over the tank or vat 2 to allow the excess material to drain from the article. Because of the rapid evaporation, this drainage period must be quite short, varying from a few seconds to ordinarily not more than a minute since the evaporation of the solvent occurs quite rapidly with deleterious effect. The drip is severed or cut, and the article inverted to allow the remaining surplus material to flow reversely over the article and redistribute itself.

The coated article is slowly revolved, preferably about an axis intersecting the article or closely adjacent thereto, so that displacement of the fluid material by centrifugal influence is minimized. By this operation the liquid material is evenly distributed over the surface of the article. While continuing the rotation, the article is immediately transferred to a refrigerating room of very much lower temperature.

In practice, articles coated with liquid material at a temperature of approximately seventy degrees Fahrenheit are transferred to a curing room wherein a temperature of approximately fifteen to twenty degrees below zero is maintained. This temperature change quite naturally causes a great increase in the viscosity of the coating material and gives it the required set, whereby it is not inclined to change its shape or position. In the curing operation, advantage is taken of two physical conditions, i. e., the lowering of the temperature causes a lowering of the vapor tension, consequently the atmosphere can contain less water vapor at the lower temperature than at a high temperature, and advantage is taken also of the latent heat of evaporation. The rotation of the article is preferably continued during the curing or drying operation within the cold room. The acetone or other solvent employed is much less volatile in the cold room, consequently the solvent escapes more slowly from the deposited material without expansion, thereby obviating the dangers of pimpling or bubbling and ballooning by which the deposit would otherwise be distorted.

Even though the temperature of the room be maintained quite low, the evaporation of the solvent nevertheless produces a refrigerating effect tending to lower the temperature of the coated article below that of the surrounding atmosphere, and thereby induce on the surface coating condensation of moisture in the form of ice crystals. This effect, however, is counteracted by extracting the

moisture from the air to a degree well below the saturation point before the air comes in contact with the coated article. To this end the curing room or cold room 3, as illustrated in the drawing, is divided by a partition 4 into two compartments which communicate with each other at the top and bottom of the wall 4. In one of these compartments 5, there are located refrigerating coils 6 by which the air currents circulating within the room 3 are cooled to approximately twenty degrees below zero. This chilling of the air causes the condensation of moisture therefrom upon the refrigerator coils 6 in the form of ice or frost, leaving the air comparatively dry, yet but little below the point of saturation of the resulting temperature. At the bottom of the compartment 5 there is located a tempering unit 7 or warming coil which slightly raises the temperature of the air after it has passed over the refrigerator coils 6. By raising the temperature of the curing air approximately five to ten degrees, that is to say, from the temperature of minus twenty to minus fifteen or minus ten Fahrenheit, not only is danger of moisture condensation by the refrigerating effect of the evaporating solvent removed, but the capability of the air to absorb the solvent vapors, which have a great affinity for moisture, is greatly increased.

The chilling of the air within the compartment 5 as it passes over the coils 6 causes a downward current of air whereas the air passing from the bottom of the compartment through the tempering unit 7, by which its temperature is raised is given a tendency to rise within the curing room 3 outside the compartment 5 to which the air returns through the space 9 above the partition 4 after passing over the coated articles being cured and absorbing therefrom the vaporized solvent. Thus the cold air descending in the compartment 5 and the slightly warmer air ascending in the room 3 induces natural convection currents affording a continuous circulation.

The slight warming of the air, after it has been lowered to such temperature as to condense its entrained moisture, so increases its capacity to absorb and retain moisture that none of the small remaining amount of moisture in the air will be condensed upon the surface of the work, which, due to the evaporating effect of the solvent, is somewhat colder than the air circulating thereabout. The low temperature retards the evaporation of the solvent, allowing sufficient time for the solvent to escape from the deposited material without causing pimples or bubbles. The subjection of the coated article to such lowered temperature also enables a heavier or deeper deposit to be retained upon the article than would otherwise be possible. Thus coverings or coatings of considerable

thickness may be effected by a single dipping operation: To afford coverings of maximum thickness, the dipping and curing operations may be repeated several times.

By rotating the article not only while transferring it from the dipping tank or vat to the chill room but during the curing process, any tendency of the material to change its position or shift upon the article is obviated. As illustrated in the drawing, a hand truck 10 equipped with an air motor 11 supplied from a pressure reservoir 12 or other suitable driving means may be provided for rotating a series of removable supporting bars 13 having thereon studs or pins 14 upon which dipped articles may be temporarily mounted. In order that the articles mounted upon these supporting bars may be rotated about axes passing thru or closely adjacent to the articles, the bars 13 are provided with terminal cranks or offset trunnions 15 about which the supporting bars and articles revolve. These supporting bars are removably engageable in a rack upon the hand truck 10 in which they are operatively connected with the driving motor for slow rotation during transference from the dipping room to the curing room. In the latter room they may be left upon the truck 10 for continued rotation, or may be transferred to a suitable rack in such room wherein the supporting bars are rotated by suitable driving means.

At 16 there is shown a revoluble bar or shaft for supporting annular coated bodies such as toilet seats. In this case a straight bar 16 extends through openings in a series of articles which are secured to arms 17 upon such bar. A toilet seat is always provided with screw holes for attachment of the hinge connection. These same holes may be utilized for attaching the seat to an arm 17 by which it is detachably connected with the rotating shaft or bar 16.

The present material must not be confused with lacquers made from cellulose base which are variously used and applied in liquid form. Such lacquers although derived from the same base to which are added various gums and solvents differ widely from the present material in character, being brittle when dry, lacking the tensile strength and durability, and can be practically applied only in thin coatings whereas the present material can be applied to form a quite thick casing or shell about the article which will be hard but tough and practically unbreakable.

Although the commercial material known as pyroxylin, pyroxyle, or pyroxyline, otherwise known specifically as celluloid, is the preferable material, the invention is not specifically limited to this material but includes other nitrocellulose derivatives having the characteristics of pyroxylin.

While the conditioning of the air in the cur-

ing room has been described as being cooled to an extreme low degree to precipitate the moisture and the temperature then raised to increase its vapor carrying capacity before it reaches the article, such air is not necessarily colder than the surface of the coated article with which the circulating air comes in contact. The evaporation of the solvent produces a refrigerating effect which tends to lower the temperature of the surface below that of the surrounding atmosphere even at the low temperature of the curing room.

The various temperatures herein mentioned are given for illustrative purposes but with no intent to arbitrarily limit this invention to such stated temperatures nor relative temperature ranges. It is to be understood that the temperature and relative variations thereof may be varied within reasonable limits to meet different conditions of use, differences in the material composition and solvent employed, and results desired.

From the above description it will be apparent that there is thus provided a method of the character described possessing the particular features of advantage before enumerated as desirable, but which obviously is susceptible of modification in its steps, sequence, detail procedure and arrangement of apparatus without departing from the principle involved or sacrificing any of its advantages.

While in order to comply with the patent statutes the invention has been described in language more or less specific as to structural features, it is to be understood that the invention is not limited to the specific details described, but that the means and method herein disclosed comprise the preferred form of several modes of putting the invention into effect, and the invention is, therefore, claimed in any of its forms or modifications within the legitimate and valid scope of the appended claims.

Having thus described my invention, I claim:

1. The herein described method of coating articles with material having a nitrocellulose base or the like, consisting in reducing the material to a semi-liquid form by the addition of a solvent, dipping the article to be coated in the liquid material at a temperature of approximately seventy degrees Fahrenheit, draining the excess therefrom, severing the drip and reversing the position of the article to redistribute the surplus material and slowly rotating the coated article to maintain distribution, transferring the coated article into a temperature of approximately minus fifteen degrees Fahrenheit and subjecting the article to the action of circulating air which has been previously chilled to approximately minus twenty degrees Fahrenheit and then warmed to approximately minus fifteen degrees Fahrenheit.
2. The herein described method of coat-

ing articles with material having pyroxylin characteristics or the like, consisting in dipping the article into a semi-liquid solution of the material, draining the excess material therefrom, subjecting the coated article to a temperature materially lower than that at which the article is dipped to effect quick congealing and retard evaporator of solvent, and drying the article at such low temperature in air from which moisture has been extracted to a degree well below the dew point at such temperature.

3. The herein described method of coating articles with material having pyroxylin characteristics or the like, consisting in dipping the article into a semi-liquid solution of the material, draining the excess material therefrom, subjecting the article to a lower degree of temperature than that at which it was dipped to effect quick congealing, and drying the coated article in an arid atmosphere to prevent condensation of atmospheric moisture thereon.

4. The herein described method of coating articles with material having pyroxylin characteristics or the like, consisting in dipping the article into a semi-liquid solution of the material, draining the excess material therefrom, rotating the coated article about an axis in proximate relation with the article to maintain distribution without displacement of the material under centrifugal influence, and curing the coated article in a cold arid atmosphere of lower temperature than that of the material in which the article was dipped whereby the solvent will be permitted to evaporate but slowly, and precipitation of atmospheric moisture will be obviated.

5. The herein described method of coating articles with material having pyroxylin characteristics or the like, consisting in dipping the article into a semi-liquid solution of the material, draining the excess material therefrom, and subjecting the article while drying to a temperature materially lower than that of the material in which it was dipped.

6. The herein described method of coating articles with material having the characteristics of pyroxylin or the like, including dipping the article into a semi-liquid solution of the material at approximately normal atmospheric temperature, and subjecting the dipped article while drying to a substantially zero Fahrenheit temperature substantially as and for the purpose specified.

7. The herein described method of coating articles with material having pyroxylin characteristics or the like, including dipping the article to be coated into a semi-fluid solution of the material, draining the excess material therefrom, and drying the article at a temperature of approximately zero Fahrenheit, in preconditioned air, the moisture content of which is lowered below the dew point at the drying temperature of the article.

8. The herein described method of coating articles with material of pyroxylin characteristics or the like, consisting in dipping the article in a semi-liquid solution of the material, draining the excess material therefrom, and drying the coated article at a substantially zero Fahrenheit temperature whereby the solvent will be maintained below boiling to prevent bubbling and pimpling and the drying will be retarded until the solvent has evaporated to prevent wrinkling.

9. The herein described method of coating articles with material of pyroxylin characteristics or the like, consisting in dipping the article in a semi-liquid solution of the material, draining the excess material therefrom, and drying the coated article at a temperature approximately seventy degrees Fahrenheit less than the temperature of the material at the time of dipping.

10. The herein described method of coating articles with pyroxylin or the like, consisting in reducing the material to semi-liquid form by the addition of a solvent, and maintained at approximately normal atmospheric temperature, dipping the article in the liquid coating material, and subjecting the coated article to a materially lower temperature by which the material is quickly congealed and loss of solvent retarded in an atmosphere from which excess moisture has been extracted.

11. The herein described method of coating articles with material having a nitrocellulose base, consisting in reducing the material to semi-liquid form by the addition of a solvent, dipping the article therein at a moderately high temperature, subjecting the dipped article to a refrigerating effect in an atmosphere wherein the moisture content is maintained materially below the point of saturation.

12. The herein described method of coating articles with a material having a nitrocellulose base, including reducing the material to a semi-liquid form by the addition of a solvent, dipping therein the article to be coated, chilling the coated article to congeal the coating material and retard evaporation of the solvent, and subjecting the article to a dry air treatment whereby condensation of moisture upon the coated surface will be obviated.

13. The herein described method of coating articles with material having a nitrocellulose base including reducing the material to a semi-liquid form by the addition of a solvent, dipping an article to be coated therein at approximately normal room temperature, subjecting the dipped article to a freezing temperature and simultaneously subjecting it to the action of air, the temperature of which has been previously lowered to a lesser degree to effect precipitation of moisture and then raised to a higher degree of temperature before reaching the coated article.

14. The herein described method of coating

articles with material having a nitrocellulose base including reducing the material to a semi-liquid form by the addition of a solvent, dipping an article to be coated therein, subjecting the dipped article to a substantially zero Fahrenheit temperature, and simultaneously circulating thereabout air from which moisture has been extracted to a point below the dew point at the temperature of the refrigerating effect produced by evaporation of the solvent from the coated article.

15. The herein described method of coating articles with material having a nitrocellulose base including reducing the material to a semi-liquid form by the addition of a solvent, dipping an article to be coated therein, subjecting the dipped article to a temperature of approximately seventy degrees (Fahrenheit) less than the temperature of the material in which it was dipped, and simultaneously drying the dipped article in air from which moisture has been extracted below the dew point at the temperature of the refrigerating effect produced by the drying of the article.

16. The herein described method of coating articles with material having a nitrocellulose base including reducing the material to a semi-liquid form by the addition of a solvent, dipping an article to be coated therein, chilling the coating material to effect congealing of the coating material prior to the escape of the solvent to prevent displacement, and subsequently removing the solvent from the congealed coating material.

17. The herein described method of coating articles with material having a nitrocellulose base including reducing the material to a semi-liquid form by the addition of a solvent, dipping an article to be coated therein, congealing the coating material prior to removal of the solvent and controlling the subsequent evaporation of solvent whereby the solvent will escape slowly.

18. The herein described method of coating articles with material having a nitrocellulose base including reducing the material to a semi-liquid form by the addition of a solvent, dipping an article to be coated therein, setting the material prior to removal of the solvent, and subsequently evaporating the solvent therefrom in an atmosphere which has been previously cooled to a degree less than that produced by the refrigerating effect of the evaporating solvent to precipitate the moisture and then rewarmed.

19. The herein described method of coating articles with material having a nitrocellulose base including reducing the material to a semi-liquid form by the addition of a solvent, dipping an article to be coated therein, congealing the material prior to the removal of the solvent and subsequently removing the solvent.

20. The herein described method of coating articles with material having a nitrocellulose

base including reducing the material to a semi-liquid form by the addition of a solvent, dipping an article to be coated therein, chilling the coating material upon the article to effect congealment thereof and evaporating the solvent therefrom at a temperature less than that at which the coating material was applied.

21. The herein described method of coating articles with material having a nitrocellulose base including reducing the material to a semi-liquid form by the addition of a solvent, dipping an article to be coated therein, subjecting the coating upon the article to a 10 congealing treatment prior to the escape of the solvent and subsequently removing the solvent sufficiently slowly to prevent bubbling, pimples or blisters in an atmosphere from which moisture has been extracted to 15 such degree as to avoid condensation at the 20 surface temperature of the coated article.

In testimony whereof, I have hereunto set my hand this 19th day of October, A. D. 1929.

WILLIAM C. HAMPTON.

25

30

35

40

45

50

55